

## UNITED STATES PATENT OFFICE

MATTHEW GREEN AND VAN M. DARSEY, OF DETROIT, MICHIGAN, ASSIGNEES TO  
PARKER RUST-PROOF COMPANY, OF DETROIT, MICHIGAN, A CORPORATION OF  
MICHIGAN

## PROCESS OF PRODUCING A PHOSPHATE COATING ON METAL

No Drawing.

Application filed April 29, 1929. Serial No. 359,166.

This invention relates to producing a phosphate coating on metal and more particularly to a method by which the desired coating can be produced quickly and economically.

The coating of iron and steel by subjecting to a dilute solution of acid phosphates and phosphoric acid has been in commercial use for many years. It is customary to prepare a phosphate bath and when properly balanced, to immerse the articles to be coated in the heated bath until complete or sufficient reaction has taken place. The action consists essentially in the combination of some of the metal on the surface of the article with phosphoric acid or acid phosphates and the forming in situ on the surface of the metal of normal or substantially insoluble phosphates. This action is normally accompanied by the release of hydrogen, and the escape of the hydrogen bubbles is some indication of the activity of the reaction. For a rust-proof coating as complete as the bath will form, the articles are left in the bath until reaction, indicated by the escape of hydrogen bubbles, has substantially ceased.

The phosphates in the bath are depleted to some extent in producing the phosphate coating upon the articles, but a large proportion of the phosphates remain in the bath after the first batch has been coated to completion, and generally a number of loads of work may be coated in succession in the same bath without replenishment. Even when the bath is so depleted that further use without replenishment is inadvisable, there still remains in the bath a large quantity of chemicals which it is inadvisable to waste. For this reason it is customary to add fresh chemicals to the bath from time to time in order to keep it up to the desired strength, and also to add water as it boils away. In this way the bath is replenished from time to time, and continues in use, without entire renewal, for long periods of time.

When a bath is first prepared from fresh chemicals, the reaction is comparatively quick. After the bath has been used and replenished for a considerable length of time in the manner described above, the time of re-action is very materially lengthened. The

bath is said to be "aged". It requires additional time or tank room, or both, to treat articles in an aged bath over what would be required in fresh solution, but in order to avoid waste of chemicals, it has been considered necessary to continue to use aged baths.

Not only is the use of an aged bath troublesome because of the increased length of time required in such a bath, but the coating is in some ways less desirable, and an article requires more careful and perfect cleaning in order to receive a satisfactory coating in an aged bath than it does in a fresh bath. The action of the aged bath is particularly slow immediately at the start of the reaction. When articles are immersed in a fresh bath, reaction at a rapid rate begins at once. When the articles are immersed in an aged bath, the reaction is comparatively slow at the start, gradually increasing to a maximum, and finally decreasing gradually until the reaction is completed.

In accordance with the present invention, there are provided two baths, a preliminary bath and a main bath. The preliminary bath is very much smaller than the main bath, and is prepared fresh with sufficient frequency to retain the characteristics of a new bath as distinguished from an aged bath. The articles are then dipped in the preliminary bath for a brief period, merely sufficient to start the reaction, and are then immersed in the main bath and coated in the usual way. The main bath is replenished from time to time in the usual manner, so that it is similar to the aged baths heretofore used.

The result of the preliminary treatment in a fresh bath is to greatly reduce the time necessary for the desired reaction in the main bath. This is true whether the articles are left in the bath to substantially complete the reaction, or whether a comparatively light coating only is produced upon the surface of the articles, suitable for receiving subsequent coatings. To mention one specific example, when the time for producing a complete coating in the main bath was upwards of an hour for articles not treated in the preliminary bath, it was found that articles given a one-minute

treatment in the preliminary bath reacted fully in the main bath in one-half hour, or less than half of the time required for the articles without such preliminary treatment. The coating produced by this half hour treatment was as satisfactory in all respects as the coating produced by the longer reaction in the same bath without the preliminary treatment.

A phosphate coating sufficient for some purposes may be produced without leaving the articles in the bath until chemical reaction ceases. In such cases, the preliminary treatment may be employed with a shortened time in the main bath. For example, where a coating sufficient for its intended use can be formed in an aged bath in one half hour, an equally good coating can be formed by a brief preliminary treatment in a fresh bath and a subsequent treatment in an aged bath not taking, together, more than fifteen minutes. This results from the fact that the preliminary treatment speeds up the first portion of treatment in the aged bath fully as much as the entire treatment.

The frequency with which the preliminary bath must be renewed depends upon the quantity of material in the bath in proportion to the amount of articles treated therein. For usual practice, it has been found that the preliminary tank may be used for one day without renewal, and that then the entire contents of the preliminary tank may be transferred to the main tank, in order to avoid wasting chemicals, and the preliminary tank may be replenished with a fresh bath. Inasmuch as the main tank must be many times the size of the preliminary tank in order to fully treat the articles, the normal boiling away of the water in the main tank leaves ample room to receive therein the entire contents of the preliminary tank as often as it is necessary to empty the preliminary tank for renewal of the bath therein.

It will be understood also that where preliminary bath and main bath are mentioned it is not necessary that the main bath be all in one tank, as it might be divided into a plurality of tanks, and the articles treated in the preliminary tank might be removed therefrom into different compartments of the main bath or in succession to one and then another of the compartments of the main bath.

The method is not limited by the examples given, for it will be understood that the length of time in the preliminary tank and the manner of maintaining a fresh solution in the preliminary tank may be varied in accordance with the requirements and exigencies of the particular case. Therefore, variations may be made within the scope of the appended claims.

What is claimed is:

1. A method of producing a phosphate coating on metal articles which comprises

providing a preliminary bath and a main bath large in proportion to the preliminary bath, first treating articles for a short time in the preliminary bath and thereafter treating said articles in the main bath for as long as is necessary to produce the desired coating, completely renewing the preliminary bath at frequent intervals, and replenishing the main bath from time to time, regardless of its aging.

2. A method of producing a phosphate coating on metal articles which comprises providing a preliminary bath and a main bath large in proportion to the preliminary bath, first treating articles for a short time in the preliminary bath and thereafter treating said articles in the main bath for as long as is necessary to produce the desired coating, transferring the preliminary bath into the main bath before the preliminary bath materially slows up in its action, and providing a fresh preliminary bath.

In testimony whereof we have hereunto signed our names to this specification.

MATTHEW GREEN. 90  
VAN M. DARSEY.

95

100

105

110

115

120

125

130